

July 5, 1938.

E. R. PIORE ET AL

2,123,024

ELECTRODE FOR ELECTRIC DISCHARGE DEVICES

Filed May 29, 1936

FIG. 1.



FIG. 2.



Inventor  
Emanuel R. Piore  
Louis Malter  
By

*J. J. Jaff*  
Attorney

## UNITED STATES PATENT OFFICE

2,123,024

## ELECTRODE FOR ELECTRIC DISCHARGE DEVICES

Emanuel R. Piore, Philadelphia, Pa., and Louis Malter, Oaklyn, N. J., assignors to Radio Corporation of America, a corporation of Delaware

Application May 29, 1936, Serial No. 82,452

5 Claims. (CL 250—27.5)

This invention relates to electric discharge devices, particularly to electrodes therefor, and has for its principal object the provision of an electrode having improved photo-sensitive and secondary-electron emissive characteristics.

Other objects will be apparent and the invention itself will be best understood by reference to the following specification and to the accompanying drawing, wherein:

10 Fig. 1 is a diagrammatic view of an electron multiplier system wherein an electrode constructed in accordance with the invention may be utilized.

Fig. 2 is a partly diagrammatic cross-sectional view greatly enlarged of a multiplying electrode constructed in accordance with the principle of the invention.

In order to increase the photo and secondary-electron emissive characteristics of certain metals, such for instance as silver, it has previously been proposed to oxidize the metal and to treat the oxidized surface with caesium, rubidium, sodium, or other electro-positive metal. A secondary-electron emissive constant of 7 to 9 is obtainable 25 with caesium on oxidized silver; rubidium on oxidized silver will provide an emissive ratio of substantially 6.5 to 8.5 secondary electrons to each impinging electron.

In constructing electrodes of the type described, 30 the preferred practice is to mount the clean metal electrode structure in the tube and, after evacuation, to introduce oxygen into the tube. The oxygen is activated or ionized, as by the application of an externally applied high frequency field and, thus activated, combines readily with the electrode metal. When oxidization has been completed the tube is re-evacuated. Caesium, which may be contained in the form of pellets within an auxiliary container connecting with 35 the tube containing the electrodes, is vaporized as by the application of heat and the resulting vapor enters into the main tube and combines with the oxidized metal to render it emissive. Excessive caesium is removed or "taken-up" within the tube. The tube is baked, on the pump, and the sealing-in operation completed.

The present invention contemplates and its practice provides a metal electrode which has not only been oxidized and treated (as with caesium) 40 but also re-oxidized and retreated with the same alkali metal. The metal whose surface is to be rendered emissive is selected from the group of metals whose oxides have a heat of formation, per oxygen bond, of the same or substantially 45 the same order as that of the metallic element

with which it is treated. Thus, whereas the prior art dictates the treatment of silver (whose oxide has a heat of formation of the order of 5000 calories per mol.) with a single application of caesium (whose oxide has a heat of formation of substantially 88,000 calories per mol.), the present invention involves a double application of caesium, or the like (with the introduction of oxygen between these applications), to a metal whose oxide has a heat of formation of the same 10 order of magnitude as that of caesium.

Among the metals whose emissive characteristics may be enhanced by the improved method of my invention are beryllium, zirconium, molybdenum, columbium and zinc. The heat of formation of the oxides, per oxygen bond, of these metals is of the order of 80,000 to 90,000 calories per mol. The alkali metals preferably employed in treating the above mentioned metals are caesium, rubidium, and potassium. The heat of 15 formation of the oxides of these metals are, respectively, 88,000, 83,500, and 86,800. Sodium whose oxide has a heat of formation of substantially 100,000 may be included in this group.

In carrying the invention into effect the electrode to be treated is first pre-oxidized, either electrolytically before it is mounted in the discharge tube, or by an oxygen glow discharge within the tube itself, or it may be oxidized within or without the tube in any known manner. Preferably this oxide coating is of a thickness of the order of, say, three hundred atomic layers. With the oxidized electrode surface or surfaces mounted within the tube, the tube is highly evacuated and a substantial amount of caesium, or like alkali metal, is distilled into it, preferably in the manner previously described. The excess caesium or other vapor is removed as by baking at a temperature of 200° F. for about ten minutes with the tube on the pump. Oxygen gas is then 25 admitted and allowed to remain in the tube for, say three minutes, until it has reacted with the caesium to form a layer of a mixture constituted of an oxide of caesium and the oxide of the metal of which the base is formed. The tube is then re-evacuated, after which the electrode is again bathed in the alkali metal vapor. This second bath of metal vapor forms a molecular layer of the alkali metal on the surface of the "mixed oxide layer". The excess metal vapor is removed 30 by baking and pumping, as before, and the tube is then sealed off.

Referring now to Fig. 1 of the drawing in which electrodes formed in accordance with the invention are utilized in an electron multiplier 35

- device of a known type. The device comprises a Y-shape evacuated container 1, within which, adjacent the closed ends of one of its arms, is mounted a photosensitive cathode 3 and adjacent the closed end of the other of its arms is an output electrode 5. A third electrode 7 is mounted between the input and output electrodes 3 and 5 in the angle or stem of the Y-shape container 1. Both electrodes 3 and 7 are constituted in accordance with the invention of a metal base having a mixed oxide coating and a layer of alkali metal superimposed on this coating. The output electrode 5 may be of nickel or other suitable material.
- 15 A variable or a constant light source may be so disposed with respect to the container that light therefrom falls upon the photosensitive cathode. In the drawing, such light source is exemplified by a lamp 8 connected in circuit with a battery 9 and a variable rheostat 11, and a lens 13.
- Under the influence of light from the source, electrons leave the surface of the photosensitive cathode in random directions. Since it is desirable to focus all such electrons upon the multiplying electrode an electromagnetic coil 15 may be disposed around one arm of the container between the photo-sensitive cathode and the multiplying electrode. A similar coil 17 may be disposed around the other arm of the container for the purpose of focusing secondary electrons upon the output electrode.
- The several focusing coils may be provided with unidirectional potential from a battery 19 or the like. In the drawing these coils are exemplified as being connected in parallel to the battery, a potential divider 21 and a plurality of contact devices 23 and 25 being utilized for the purpose of individually controlling the magnitude of the several focusing field currents. It is our understanding that the polarity of the coils is immaterial. Alternatively, electrostatic focusing of the electrons may be resorted to, or a combination of electrostatic and magnetic focusing.
- 45 In the operation of an electron multiplier of the type under discussion the output electrode 5 may be connected to any suitable utilization circuit, such as a relay 27. When utilizing a multiplier of the type shown, the photosensitive-cathode 50 may be connected to the negative terminal of a potential divider 29 that is connected across a source of unidirectional potential 31, the output electrode 5 connected to the positive terminal of the potential divider and the multiplying electrode 55 7 connected to an intermediate point thereon. The relative potentials shown in the drawing are to be construed solely as illustrative.

Referring to Fig. 2, the base upon which the mixed oxide layer and the alkali metal coating is applied may be a mere sheet of beryllium intimately jointed, as by evaporation, to a base of another and cheaper metal, such for instance as 5 nickel. Such construction is recommended where the metal to which the mixed oxide layer and alkali metal coating is applied is not available in sheet form.

As indicated in both Figs. 1 and 2, when the 10 electrons constituting the primary beam from the cathode strike the composite electrode surface with sufficient energy, secondary-electrons are emitted. The electrons, so released are drawn to the collector electrode, or if desired to another 15 similar surface for further multiplication by reason of the electric field applied between the emitter and the target electrode.

While the invention has been described in connection with a photo-actuated electron-multiplier tube, it is to be understood that its application is not to be limited to the particular type of tube here described, as the disclosure, in this respect, is merely illustrative for purposes of explaining the inventive concept. 25

What is claimed is:

1. An electrode comprising a metal base having thereon a layer of a mixture of an oxide of said metal and an oxide of an alkali metal whose oxide has a heat of formation, per oxygen bond, 30 of substantially the same order as that of the oxide of the metal constituting said base, and a coating of said alkali metal superimposed on said layer.
2. An electrode comprising a base of a metal 35 whose oxide has a heat of formation, per oxygen bond, of the order of substantially 80,000 to 90,000 calories per mol., a layer on said base constituted of an oxide of said metal and an oxide of an alkali metal whose oxide has a heat of formation, 40 per oxygen bond, of the order of substantially 80,000 to 100,000 calories per mol., and a surface coating of said alkali metal on said layer.
3. An electrode comprising a base of beryllium, a layer on said base constituted of beryllium and 45 caesium oxides and a surface coating of caesium on said layer.
4. An electrode comprising a base of beryllium, a layer on said base constituted of beryllium and rubidium oxides and a surface coating of rubidium 50 on said layer.
5. An electrode comprising a base of beryllium, a layer on said base constituted of beryllium and potassium oxides and a surface coating of potassium on said layer.

EMANUEL R. PIORE.  
LOUIS MALTER.